

## [54] ANODE COMPOSITIONS

[75] Inventors: **Edgar J. Seyb**, Oak Park; **Melvyn B. Kalt**, Royal Oak; **Hyman Chessin**, Birmingham, all of Mich.

[73] Assignee: **M & T Chemicals Inc.**, New York, N.Y.

[22] Filed: **Nov. 5, 1971**

[21] Appl. No.: **196,206**

**Related U.S. Application Data**

[62] Division of Ser. No. 830,851, June 5, 1969, abandoned.

[52] U.S. Cl. .... **204/51, 204/293**

[51] Int. Cl. .... **C23b 5/06, B01k 3/06**

[58] Field of Search. .... **204/51, 293**

[56] **References Cited****UNITED STATES PATENTS**

|           |         |                   |       |          |
|-----------|---------|-------------------|-------|----------|
| 1,766,871 | 6/1930  | Beckinsale et al. | ....  | 75/166 C |
| 2,060,534 | 11/1936 | Singleton et al.  | ....  | 75/166 R |
| 2,841,541 | 7/1958  | Smith             | ..... | 204/51   |
| 2,729,602 | 1/1956  | Van Houton        | ..... | 204/55 R |

**FOREIGN PATENTS OR APPLICATIONS**

508,604 7/1939 Great Britain ..... 75/166 B

**OTHER PUBLICATIONS**

Transactions of the Electrochemical Soc., Vol. 80, pp. 59 and 60 by Bray et al., 1941.

*Primary Examiner*—F. C. Edmundson

*Attorney*—Lewis C. Brown, Kenneth G. Wheless et al.

[57] **ABSTRACT**

In accordance with certain of its aspects, this invention relates to novel processes and to a lead base alloy suitable for anode production consisting essentially of lead and tin and at least one metal selected from the group consisting of tellurium, thallium, and cadmium and containing 90-99 percent by weight of lead, 1-7 percent by weight of tin, and at least one metal selected from the group consisting of tellurium, thallium, and cadmium in an amount of 0.005-5.0 percent by weight sufficient to bring the total weight of the lead base alloy anode to 100 percent.

**9 Claims, No Drawings**

## ANODE COMPOSITIONS

This application is a divisional application of Ser. No. 830,851, filed June 5, 1969, now abandoned.

This invention relates to novel anodes, novel anode compositions, and to the preparation of such anodes and their use in electroplating processes. More particularly, this invention relates to the preparation and use of novel lead base alloy anodes containing 90-99 percent by weight of lead, 1-7 percent by weight of tin, and at least one metal selected from the group consisting of tellurium, thallium, and cadmium in amounts sufficient to bring the total weight of the lead base alloy anode to 100 percent by weight.

Lead anodes are known to be useful in chromium electroplating baths and various alloys have been used in the past with varying degrees of success. Attempts have been made to modify the shapes of such anodes in order to provide anodes which carry a higher surface current density than conventional anodes of equal cross-sectional area and to reduce the build-up upon the anode of undesirable deposits such as chromate deposits. During the course of chromium plating operations, lead anodes become heavily coated with lead oxides (mainly lead dioxide,  $PbO_2$ ). When left standing in a solution containing chromic acid, a lead anode ordinarily becomes coated with lead chromate and such coatings act to partially insulate the anode, thus interfering with the normal distribution of the chromium deposited on the cathode. Such defects are especially undesirable in industrial chromium plating where irregularities in current distribution may produce wide variations in chromium plate thicknesses. During conventional operations, therefore, it may become necessary to remove such incrustations from conventional lead anodes by wire brushing or by chemical treatment using solutions containing hydrochloric acid or aqueous solutions containing alkali-metal pyrophosphate or other cleaning agents.

It is an object of the present invention to provide an improved lead alloy anode which is essentially free of antimony, bismuth, and arsenic. Another object of the invention is to provide an improved chromium electroplating process using a lead base alloy anode which is particularly resistant to attack by chromic acid. A further object of the invention is to provide a lead base alloy anode which gives superior chromium electrodeposits and is characterized by particularly long life when subjected to the corrosive attack of chromic acid and other chromium plating bath chemicals.

In accordance with certain of its aspects, this invention relates to novel processes and to a lead base alloy suitable for anode production consisting essentially of lead and tin and at least one metal selected from the group consisting of tellurium, thallium, and cadmium and containing 90-99 percent by weight of lead, 1-7 percent by weight of tin, and at least one metal selected from the group consisting of tellurium, thallium, and cadmium in an amount of 0.005-5.0 percent by weight sufficient to bring the total weight of the lead base alloy anode to 100 percent.

The lead base alloy anodes of the invention are particularly characterized by the substantial absence of antimony, bismuth, and arsenic from the alloy. The lead base alloy anodes of the invention are preferably at least ternary alloys consisting essentially of lead, tin, and tellurium or thallium, or cadmium, or combinations of one or more of these last three metals. Typical

lead base alloy anodes may about 90-98 percent by weight of lead, about 2-5 percent by weight of tin, and the remainder tellurium (typically in amounts sufficient to saturate the alloy) or thallium (typically in amounts up to 1 percent by weight), or cadmium (typically in amounts up to 2 percent by weight). Higher percentages of tin, tellurium, thallium, or cadmium may be used according to the invention, but cost considerations generally do not justify the use of excessive amounts of these metals.

The lead base alloy anode compositions are prepared by melting the metals together or by adding and dissolving the metals for a particular alloy in molten lead and then cooling the resulting lead base alloy anode composition.

The lead base alloy anodes prepared according to the invention have good hardness properties, excellent electrical properties (including good initial resistance during start up periods in chromium plating process) and are particularly resistant to attack by chromic acid during the chromium electroplating process. The lead base alloy anodes are exceptionally resistant to attack in chromic acid which contains additives such as sulfates, fluorides, and especially mixed radicals such as sulfate  $SO_4^{2-}$  and silicofluoride  $SiF_6^{2-}$ .

Typical lead alloy anode compositions which may be employed according to the invention and which have been found superior to prior art lead base anodes include the following examples which are summarized in Table I. In Table I all parts are given in percent by weight based upon the total weight of the lead base alloy.

TABLE I

| Metal                | Amount<br>(Percent by Weight) |     |
|----------------------|-------------------------------|-----|
|                      | 90-99                         | 1-7 |
| (1) Lead             |                               |     |
| (2) Tin              |                               |     |
| and at least one of: |                               |     |
| (3)                  |                               |     |
| a. Tellurium         | 0.000 - 0.05                  |     |
| b. Thallium          | 0.000 - 1.00                  |     |
| c. Cadmium           | 0.000 - 2.00                  |     |

## Typical Lead Base Alloy Anode Compositions

|           | A     | B     | C     | D     | E     | F     |
|-----------|-------|-------|-------|-------|-------|-------|
| Lead      | 97.97 | 97.00 | 95.00 | 97.00 | 96.25 | 96.00 |
| Tin       | 2.00  | 2.25  | 2.50  | 2.00  | 3.00  | 2.00  |
| Tellurium | 0.03  | 0     | 0     | 0.02  | 0.03  | 0.01  |
| Thallium  | 0     | 0.75  | 0     | 0.03  | 0.72  | 0     |
| Cadmium   | 0     | 0     | 2.50  | 0.95  | 0     | 1.99  |

Typical chromium plating baths in which the lead base alloy anode compositions of the invention may be employed may contain from about 150-600 g/l of chromic acid (as  $CrO_3$ ). Illustrative acidic aqueous chromium plating baths which may be employed include the following bath compositions:

| Component                                     | Amount<br>g/l | Preferred<br>Concentrations<br>g/l |
|-----------------------------------------------|---------------|------------------------------------|
| I Chromic acid                                | 150-600       | 250                                |
| Sulfate ion<br>(e.g. from sulfuric acid)      | 1-10          | 2.5                                |
| II Chromic acid                               | 150-600       | 250                                |
| Sulfate ion<br>(e.g. from sulfuric acid)      | 0.5-5         | 1                                  |
| Silicofluoride ion<br>(e.g. from $H_2SiF_6$ ) | 1-10          | 2                                  |
| III Chromic acid                              | 150-600       | 400                                |
| Sulfate ion<br>(e.g. from strontium sulfate)  | 1-5           | 2                                  |
| Silicofluoride ion<br>(e.g. from $H_2SiF_6$ ) | 2-8           | 5                                  |

Another aspect of the invention relates to a process for electrodepositing chromium from an aqueous acidic chromium electroplating bath which contains at least one chromium compound providing chromium metal ions for electroplating chromium which comprises passing current from a lead base alloy anode consisting essentially of lead, tin, and at least one metal selected from the group consisting of tellurium, thallium,

5 was greater than 0.50 grams per square centimeter were classified as poor. As can readily be seen from Table II, lead base alloy anode compositions prepared in accordance with the invention herein showed good resistance to attack in chromic acid solutions. In addition, the lead base alloy anode compositions of the invention possess excellent initial-resistance characteristics and provide excellent chromium plated articles.

TABLE II  
Lead Base Alloy Anode Compositions

| Ex. No.                                        | 1      | 2      | 3      | 4      | 5      | 6      | 7      | 8      | 9<br>Control |
|------------------------------------------------|--------|--------|--------|--------|--------|--------|--------|--------|--------------|
| (Percent by Weight)                            |        |        |        |        |        |        |        |        |              |
| Metal                                          |        |        |        |        |        |        |        |        |              |
| Pb                                             | 97.95  | 96.0   | 97.0   | 96.995 | 94.0   | 96.225 | 94.525 | 94.50  | 100.0        |
| Sn                                             | 2.0    | 2.0    | 2.0    | 2.0    | 3.0    | 3.0    | 4.0    | 4.0    | 0            |
| Te                                             | 0.05   | 0      | 0      | 0.005  | 0      | 0.025  | 0.025  | 0.05   | 0            |
| Tl                                             | 0      | 0      | 1.0    | 0.5    | 1.0    | 0.75   | 0      | 0.50   | 0            |
| Cd                                             | 0      | 2.0    | 0      | 0.5    | 2.0    | 0      | 1.450  | 0.95   | 0            |
| TOTAL                                          | 100.00 | 100.00 | 100.00 | 100.00 | 100.00 | 100.00 | 100.00 | 100.00 | 100.00       |
| Anode<br>Weight<br>Loss<br>G./cm. <sup>2</sup> | 0.27   | 0.22   | 0.27   | 0.25   | 0.20   | 0.22   | 0.19   | 0.20   | 0.79         |

and cadmium, wherein said lead base alloy anode contains 90-99 percent by weight lead, 1-7 percent by weight tin, and the remainder of said lead base alloy anode consists of at least one metal selected from the group consisting of tellurium, thallium, and cadmium to a cathode through said aqueous acidic chromium plating solution to produce a chromium surface on at least a portion of said cathode.

Chromium electroplating is ordinarily carried out with the novel lead base alloy anode of the invention using bath temperatures of 15°-95° C. and plating currents of 1-60 amperes per square decimeter (asd).

The following examples are submitted for the purpose of illustration only and are not to be construed as limiting the scope of the invention in any way.

#### GENERAL PROCEDURE

Lead base alloy anodes were prepared by melting the indicated amounts of lead and tin together and then adding the indicated amount of tellurium, thallium, and cadmium to obtain a metal solution. The so-formed alloy was then cast into cold molds or extruded to the desired shape of the anode.

All of the lead base alloy anode compositions described in the illustrative examples possess superior hardness and resistivity against attack from chromic acid solutions when compared with the control anodes.

Resistance to chromic acid attack was measured by immersing an anode into a solution of chromic acid containing 240 g/l of chromic acid and the mixed radicals, sulfate, and silicofluoride at a temperature of 43° C. for a time of 120 hours. During this time the solutions were electrolyzed with an anode current density of 20 amperes per square decimeter (asd) for eight hour periods and then let stand for 16 hours. At the end of 120 hours, the anodes were removed and the weight loss of each determined. The loss of anode weight was measured after removal of deposits formed on said anode by side reactions such as the reaction of the anode with the chromic acid. Anodes wherein the loss of anode material was less than 0.35 grams per square centimeter of immersed anode surface were considered good and anodes wherein the loss of anode material

35 Another control consisting of a binary alloy containing 90 percent Pb and 10 percent Sb exhibited a corresponding loss of 0.70 g/cm<sup>2</sup>.

As can be seen from Table II, lead-base alloy anodes 30 of the invention possess good resistance to attack in chromic acid solutions.

Although this invention has been illustrated by reference to specific embodiments thereof, numerous modifications which are clearly within the scope of the invention will be apparent to those skilled in the art.

We claim:

1. A process for electrodepositing chromium from an aqueous acidic chromium electroplating bath which 40 contains at least one chromium compound providing chromium metal ions for electroplating chromium which comprises passing current from a lead base alloy anode consisting essentially of lead, tin, and at least one member selected from the group consisting of tellurium, thallium, and cadmium, wherein said lead base alloy anode contains 90-99 percent by weight lead, 1-7 percent by weight tin, and the remainder of said lead base alloy anode consists of at least one member selected from the group consisting of tellurium, thallium, 45 and cadmium to a cathode through said aqueous acidic chromium plating solution to produce a chromium surface on at least a portion of said cathode.

2. A process as claimed in claim 1 wherein the chromium electroplating bath contains sulfate  $\text{SO}_4^{2-}$  and 55 silicofluoride  $\text{SiF}_6^{2-}$ .

3. A process as claimed in claim 1 wherein the lead base alloy anode contains 0.000-0.05 percent tellurium.

4. A process as claimed in claim 1 wherein the lead 60 base alloy anode contains 0.000-1.0 percent thallium.

5. A process as claimed in claim 1 wherein the lead base alloy anode contains 0.000-2.0 percent cadmium.

6. A process as claimed in claim 1 wherein the lead base alloy anode contains 0.000-0.05 percent tellurium 65 and 0.000-1.0 percent thallium.

7. A process as claimed in claim 1 wherein the lead base alloy anode contains 0.000-0.05 percent tellurium and 0.000-2.0 percent cadmium.

8. A process as claimed in claim 1 wherein the lead base alloy anode contains 0.000-1.0 percent thallium and 0.000-2.0 percent cadmium.

9. A process as claimed in claim 1 wherein the lead

base alloy anode contains 0.000-0.05 percent tellurium, 0.000-1.0 percent thallium, and 0.000-2.0 percent cadmium.

\* \* \* \* \*